

# United States Patent

[11] 3,591,955

|                |                                                                                                                                                                                                  |
|----------------|--------------------------------------------------------------------------------------------------------------------------------------------------------------------------------------------------|
| [72] Inventors | Shiro Fujita<br>Tokyo;<br>Jusuke Ushiki, Isezaki-shi; Nagao<br>Nishizawa, Matsudo-shi; Seiji Okawa,<br>Warabi-shi; Kunio Sekiya, Matsudo-shi;<br>Hiroshi Kadokawa, Matsudo-shi, all of,<br>Japan |
| [21] Appl. No. | 835,553                                                                                                                                                                                          |
| [22] Filed     | June 23, 1969                                                                                                                                                                                    |
| [45] Patented  | July 13, 1971                                                                                                                                                                                    |
| [73] Assignee  | Nippon Rayon Co. Ltd.<br>Tonouchi Uji-Uji-shi, Japan                                                                                                                                             |
| [32] Priority  | June 27, 1968, June 27, 1968                                                                                                                                                                     |
| [33]           | Japan                                                                                                                                                                                            |
| [31]           | 43/44691 and 43/44692                                                                                                                                                                            |

[51] Int. Cl. . . . . D02g 1/16,  
D02g 3/34  
[50] Field of Search. . . . . 57/34 B,  
157 F, 140 J, 91; 28/1.4, 72.12

| [56] References Cited |                               |
|-----------------------|-------------------------------|
| UNITED STATES PATENTS |                               |
| 3,118,269             | 1/1964 Bilsky .....           |
| 3,262,177             | 7/1966 Cobb et al. .....      |
| 3,296,785             | 1/1967 Hardy.....             |
| 3,433,007             | 3/1969 Myers.....             |
| 3,517,498             | 6/1970 Burellier et al. ..... |

*Primary Examiner—John Petrakes  
Attorney—Pierce, Scheffler & Parker*

[54] **PROCESS FOR PRODUCING A SLUB YARN**  
7 Claims, 13 Drawing Figs.

[52] U.S. CL..... 57/157,  
28/1.4, 28/72.12, 57/34, 57/140

**ABSTRACT:** A process for producing slubs onto a multifilament yarn which comprises feeding the yarn into a hood receiving a jet of compressed gas and withdrawing the yarn through a hole of the hood from the deflected stream of the gas at lower rate than the feed rate.



PATENTED JUL 13 1971

3,591,955

SHEET 1 OF 8

Fig. 1



PATENTED JUL 13 1971

3,591,955

SHEET 2 OF 8

Fig. 2



PATENTED JUL 13 1971

3,591,955

SHEET 3 OF 8

Fig. 3



PATENTED JUL 13 1971

3,591,955

SHEET 4 OF 8

*Fig. 4*



PATENTED JUL 13 1971

3,591,955

SHEET 5 OF 8

*Fig. 5*



*Fig. 6*



*Fig. 7*



*Fig. 8*



PATENTED JUL 13 1971

3,591,955

SHEET 6 OF 8

Fig. 9



PATENTED JUL 13 1971

3,591,955

SHEET 7 OF 8

*Fig. 10*



*Fig. 11*



PATENTED JUL 13 1971

3,591,955

SHEET 8 OF 8

Fig. 12



Fig. 13



## PROCESS FOR PRODUCING A SLUB YARN

## BACKGROUND OF THE INVENTION

It has long been known that a multifilament yarn can be slubbed by passing through a high-velocity stream of compressive fluid. In the presently known process a jet of fluid is used to introduce coils, loops and folds along the filaments forming the yarn. In any one of these process, the jet is not effectively and economically used but has been required to provide otherwise a slub jet for a sole purpose of forming the slubs. This imposes a high-consumption of the compressive fluid and high maintenance costs upon the operation, rendering the products very expensive.

The present invention is directed to eliminate the conventional slub jet by substituting deflected flow of the supply jet for the slub jet. After extensive investigation, we have found a novel method involving a hood which enables the supply jet to serve also as a slubbing jet after it is deflected at the apex of the hood.

It is the object of the present invention to provide a novel method for producing a multifilament slub yarn, according to a simple process which avoids the necessity of a slub jet.

Another object of the present invention is to provide a slub yarn in which slubs are tightly formed by continuous filaments at irregular intervals in its length.

## SUMMARY OF THE INVENTION

According to the invention, there is provided a process for producing a slub yarn characterized by:

- a. jetting a compressive gas into a hood having a hole at the apex thereof to deflect at the apex and to escape backwardly,
- b. feeding a multifilament yarn in the deflected stream of gas to fold back the filaments composing the yarn on themselves at the apex of the hood, and
- c. withdrawing the yarn from the deflected stream of gas through the hole of the hood, at a rate at least 0.5 percent less than the rate of feed, so that the yarn passes through the deflected stream of gas in a countercurrent direction to form slubs composed of filament loops consolidated into the yarn by filament entanglement.

## BRIEF DESCRIPTION OF THE DRAWING

FIG. 1 schematically shows a preferred embodiment of the apparatus for carrying out the process according to the present invention.

FIG. 2 shows a perspective view of the hood in FIG. 1 partially cut away to illustrate its inner configuration and slubbing.

FIG. 3 schematically shows another type of apparatus for carrying out the process according to the invention.

FIG. 4 shows a cross-sectional view taken along IV-IV line of FIG. 9.

FIGS. 5 to 8 show schematically broken, side views greatly enlarged of slub yarns which can be produced in accordance with the invention.

FIG. 9 shows schematically another type of the apparatus for carrying out the process according to the invention.

FIG. 10 and FIG. 11 schematically and partially shown broken, perspective views of the hoods.

FIG. 12 schematically shows an embodiment of the moving means.

FIG. 13 schematically shows main parts of a jet loom used for weaving the slub yarn.

## DESCRIPTION OF THE PREFERRED EMBODIMENTS

referring to FIG. 1 there is shown a preferred embodiment of the apparatus for carrying out the process according to the invention.

The multifilament yarn 1 is withdrawn from a letoff package 2 through pigtail guide 3 and tension disc 4, by a pair of feed

rolls 5 and 6, the yarn passing a sufficient number of times around the pair of rolls to provide positive control of the feed rate. The yarn then enters into nozzle 7 through its hole 8 and advances toward the dome-shaped apex of hood 9 with a high-velocity stream of gas introduced into the rear end of the nozzle by pipe 10. The stream of gas flowing along one side of the hood due to the fact that the longitudinal axis of the straight nozzle 7 is offset from the longitudinal axis of the hood on which the yarn withdrawal hole 16 is located is deflected along the concave surface of the apex and escapes backwardly. After deflection, the stream of gas serves to slub the yarn passing in countercurrent direction.

The yarn is then dashed against the apex of the hood by the stream and the excess length of overfeed is then folded back on the subsequently continuing portion of the yarn by the deflection of the stream. It will be understood that a certain continuance of this state might eventually allow time for forming a slub with each filament in entanglement. The slub thus produced is then withdrawn through the hole 16 at the apex by withdrawal rolls 11 and 12 similar to feed rolls 5 and 6, but operated at lower speed. The yarn passes after leaving the withdrawal rolls to a conventional windup, such as a package 13 surface driven by a takeup roll 14 through traverse guide 15.

In FIG. 2, the hood is shown in greatly enlarged state. The filaments are folded back on themselves by the deflected stream of gas. Although both feed and withdrawal are kept at constant speed during the operation, formation of slubs arises intermittently. As a result of this the portion of the yarn between the feed roll and withdrawal roll is subjected to a fluctuation of tension during the operation. The excess length of the overfeed should be controlled in a range that the overfeed is quite sufficient to insure in the yarn always necessary folds of filaments to produce the slub, but under all circumstances opposes a minimum obstruction to a stoppage of advancement into which an extremely excess feeding will fall.

Referring to FIG. 3, there is combined a fluid false twister 17 with the apparatus as described above. The other parts except the false twister are similar to corresponding parts of the apparatus of FIG. 1. The fluid false twister has fluid conduits 18 and 19, entering a cylindrical yarn passage way 20 from opposite sides as shown in FIG. 4. The fluid conduits 18 and 19 are secured to the body in tangential relationship with respect to the section of the yarn passageway, whereby a vortex stream exerted along the direction of the arrow introduces an alternate twist in the yarn. An enlarged illustration of the slub produced by the practice of the invention is shown in from FIG. 5 to FIG. 8. A state of the slub immediately after leaving the hood is seen in FIG. 5, which varies to a state of FIG. 6 by passing through the fluid false twister 17. It will be seen that the left side portion of the slub has an S twist, while the right side portion has a Z twist.

Referring to FIGS. 10 and 11, there are shown two types of the hole of the hood. The hole 16' of FIG. 10 has a recess closely neighboring with the hole which recess increases its depth to an increasing degree of approach to the hole. This serves to control the direction of the deflected stream and formation of slub is attained in a somewhat greater complication of loops of the filament than is formed by the hood having the hole 16 as shown in FIG. 11.

In FIG. 9, there is provided a yarn-scrubbing device 21 in which three poles 22 are secured on a body 23 in parallel with each other and two separators 24 are secured in contact with two neighboring poles. The yarn passes through a reverse curve formed by the poles in frictional contact with the poles under urging of the withdrawal rolls. By passing through the device, the slubs are leaned in adverse direction against the advancement of the yarn as shown in FIG. 7. The yarn shown in FIG. 8 is a product obtained by passing through both the scrubbing device and fluid false twister in this order.

In FIG. 12, is shown an eccentric disc 25, moving friction means, which serves as a false twister. The shaft 26 is mounted eccentrically to the disc. The yarn running along the shaft in-

3 intermittently and frictionally contact with the surface of the disc as the disc rotates, gaining an alternate twist in its length. The disc may be substituted for the fluid false twister for the purpose of practicing the invention.

FIG. 13 schematically and partially shows one type of jet loom for weaving the slab yarn as a weft. The slab yarn is supplied from a supply package 27 through guide 28 and 29, tensor 30, guide 31, and a pair of feed rolls 32 and 33 to pool pipe 34. The yarn is then withdrawn from the pool pipe 34, and the yarn passes through a pair of nip members 35. The yarn then is jetted with water by the nozzle 36. The nip members intermittently nip the slab yarn in accordance with a jetting cycle.

When the multifilament yarn is overfed into the deflected stream flowing backwardly from the apex of the hood, the numerous filaments forming the yarn are separated in any number of groups which are simultaneously folded back on themselves with each group in an entanglement. It is found that an irregularity of intervals of the slubs results on the yarn from a cooperation between the yarn's overfeed and passage in adverse direction against the flow of the deflected stream of the gas. It is noted that such irregular characteristic is essential to make the resultant yarn applicable in the commercial field.

The phenomenon from which the formation of the slab is achieved is not formulated, but it is our belief that there are various factors by which the formation of the slab is controlled, such as, for example, a pressure of the compressive gas, configuration or size of the hood, overfeed ratio of the yarn, and the like. We suppose that the most essential factor to acquire the irregular characteristic is the passage of the yarn through the deflected stream of the gas in countercurrent direction against the flow of the jet.

Various values in the undergoing specification have therefore been elected after extensive experiments.

Any type of hood will sufficiently be employed for the purpose of practicing the present invention, so far as desired deflection of the stream is obtained. It is preferred that the inner surface of the hood, at least the surface in the vicinity of the apex, is smoothly curved to insure the stream an efficient flowing and deflection. It is also found that the compressive gas is jetted in the chamber of the hood and the centerline of the jetted stream of gas is offset from the central, i.e. longitudinal axis of the hood.

Any kind of gas may be used in practicing the invention, if it is harmless and the pressure of the jet is controlled in a range of from 0.5-5 Kg./cm.<sup>2</sup> under a guage pressure. This range is not severe and a latitude should be permitted in a somewhat lower range than 0.5 Kg./cm.<sup>2</sup>. In view of ready availability and lower cost, air is beneficially selected for the practice of the invention.

Although the overfeed length of the yarn is found applicable in the range of 0.5-50 percent relative to the withdraw, the range of about 2-10 percent is found beneficial.

As used herein, overfeed is defined as:

$$\text{overfeed} = \frac{\text{feed rate} - \text{withdrawal rate}}{\text{withdrawal rate}} \times 100$$

It will be obvious that the yarn may be supplied to the deflected stream either directly or otherwise through a jetting nozzle and one or more of a plurality of yarns may be used in doubled state to acquire a particular effect on the resultant yarn. In this practice, any one or more of them may be supplied separately from the other by passing through the jetting nozzle or not.

A false twisting has been found advantageous in combining with the procedure above described for the purpose of gaining a consolidation of the slubs.

As the false twister, a vortex stream of gas may be utilized to impart a false twist to the yarn after leaving the hood. By this, a greater tightness and consolidation can be attained as to the slab forming. The pressure of the vortex gas is regulated in the range of about 0.5-5 Kg./cm.<sup>2</sup>.

Any other type of false twister, such as friction disc, may be used for the same purpose.

By the false twist, cohesion between filaments is beneficially obtained, opposing an obstruction to a weaving trouble. It should be noted that the true twist which may have been imparted in the slab yarn will fall into the breakage as would defeat the purpose of weaving yarn.

In the following examples and tables, the degree of the stability of slubs is designated as  $\bar{d}$  value (a low  $\bar{d}$  value means a high stability), which is determined in the following manner.

A sample yarn of 20 centimeters length having one slab in its length was supported horizontally in a tension state by fixing at both ends. A weight of (deniers of monofilament  $\times$  0.01) grams was then suspended by one of a plurality of loops of the slab by means of hanger hook. After sufficiently allowing the loop to loose by the load of the weight, an amount of a downward shift exhibited by the weight was measured. The same tests were repeated 200 times as to the sample yarns of the same nature. From the obtained values, there was yielded an arithmetic mean value representing  $\bar{d}$  value.

As shown in Table 1, several embodiments of the hood according to the invention was used in the examples.

TABLE 1

|   | 1       | 2    | 3   | 4  | 5 |
|---|---------|------|-----|----|---|
| A | Ellipse | 5.0  | 1.5 | 12 |   |
| B | do      | 5.0  | 1.5 | 15 |   |
| C | do      | 5.0  | 1.5 | 20 |   |
| D | do      | 10.0 | 3.0 | 15 |   |
| E | do      | 2.5  | 1.0 | 6  |   |

## Note:

1. Type of hood
2. Cross-sectional shape at open end of hood
3. Length of maximum axis of the ellipse, centimeters
4. Length of minimum axis of the ellipse, centimeters

## EXAMPLES 1 TO 3

Examples 1 to 3 respectively were carried out to produce a slab yarn by using embodiments of the apparatus similar to the apparatus of FIG. 1. The operational conditions are shown in Table 2 and the results obtained are given in Table 3.

## EXAMPLES 4 TO 9

Examples 4 to 9 respectively were carried out to produce slab yarn by using different embodiments of the apparatus, each of which is substantially similar to the embodiment of FIG. 1 except that each is provided with a yarn scrubbing device 17.

## EXAMPLES 10 TO 12

Examples 10 to 12 respectively were carried out to produce a slab yarn by using embodiments of the apparatus, each of which is substantially similar to the embodiment of FIG. 3.

## EXAMPLES 13 TO 17

Examples 13 to 17 were respectively carried out to produce a slab yarn by using different embodiment of the apparatus, each of which is substantially similar to the embodiment shown in FIG. 9.

## EXAMPLE 18

Example 18 was carried out to produce a slab yarn by using an embodiment of the apparatus which is similar to the embodiment shown in FIG. 9 except that it is provided with a rotatable eccentric disc used were as follows:

Diameter of disc: 10 centimeters

Distance between center of disc and center of shaft: 1 centimeter

Material of friction surface: Polyurethane rubber

Rotating speed of friction means: 3,000 r.p.m.

TABLE 2. EXAMPLES OF PROCESS CONDITIONS

| Example No. | A                                   | B   | C   | D   | E   | F  | G   | H   |
|-------------|-------------------------------------|-----|-----|-----|-----|----|-----|-----|
| 1           | Polyethylene oxybenzoate (150/48)   | 208 | 200 | 1.0 | A   | 4  | 0.5 |     |
| 2           | do                                  | 206 | 200 | 1.0 | A   | 4  | 0.5 |     |
| 3           | Polyethylene oxybenzoate (100/48)   | 240 | 200 | 1.0 | A   | 4  | 0.5 |     |
| 4           | Polyethylene oxybenzoate (150/48)   | 312 | 300 | 1.5 | C   | 4  | 0.5 |     |
| 5           | do                                  | 303 | 300 | 5.0 | C   | 4  | 0.5 |     |
| 6           | do                                  | 303 | 300 | 0.5 | C   | 4  | 0.5 |     |
| 7           | Nylon 6 (70/24)                     | 208 | 200 | 1.2 | B   | 3  | 0.5 |     |
| 8           | do                                  | 208 | 200 | 1.2 | B   | 10 | 0.5 |     |
| 9           | Polyethylene oxybenzoate (70/36)    | 204 | 200 | 1.5 | A   | 4  | 0.5 |     |
| 10          | Polyethylene oxybenzoate (100/48)   | 184 | 180 | 1.5 | 1.0 | A  | 4   | 0.5 |
| 11          | do                                  | 184 | 180 | 1.5 | 0.5 | A  | 4   | 0.5 |
| 12          | do                                  | 184 | 180 | 1.5 | 4.5 | A  | 4   | 0.5 |
| 13          | Polyethylene terephthalate (150/48) | 186 | 180 | 3.0 | 1.5 | A  | 4   | 1.0 |
| 14          | do                                  | 200 | 180 | 3.0 | 1.5 | A  | 4   | 1.0 |
| 15          | Viscose rayon (600/100)             | 159 | 150 | 3.0 | 2.0 | D  | 6   | 2.0 |
| 16          | Nylon 6 (70/24)                     | 204 | 200 | 1.5 | 1.0 | E  | 2   | 0.5 |
| 17          | Cellulose acetate (150/50)          | 204 | 200 | 1.5 | 0.5 | A  | 2   | 0.5 |
| 18          | Polyethylene oxybenzoate (150/48)   | 210 | 200 | 1.5 | A   | 4  | 0.5 |     |

## Note:

- A. Type of yarn treated (total denier/filaments)
- B. Feed speed of yarn (meter per minute)
- C. Withdrawal speed of yarn (meter per minute)
- D. Pressure of compressive air used for deflected stream (Kg./cm.<sup>2</sup>)
- E. Pressure of compressive air used for vortex (Kg./cm.<sup>2</sup>)
- F. Type of hood
- G. Distance from top end of nozzle to bottom of hood (centimeter)
- H. Distance from center of nozzle to central axis of hood
  - 1. Center axis of nozzle used was in parallel with axis of hood
  - 2. Nozzle was located on the maximum axis of the elliptical section of the hood in examples except Example 9
  - 3. Nozzle was located on the minimum axis of the elliptical section of the hood in Example 9

TABLE 3.--CHARACTERIZATION PARAMETERS OF VARIOUS SLUB YARNS

| Slub characterization parameters                         | 1   | 2   | 7   | 9   | 10  | 15  | 16  | 18  |
|----------------------------------------------------------|-----|-----|-----|-----|-----|-----|-----|-----|
| Average slub length, cm.                                 | 3.5 | 3.0 | 3.7 | 2.8 | 3.3 | 4.1 | 1.8 | 3.6 |
| Slubs/100 meters                                         | 49  | 43  | 32  | 28  | 45  | 184 | 97  | 52  |
| Longest slub in samples analyzed, cm.                    | 8   | 9   | 11  | 4   | 9   | 14  | 6   | 10  |
| Shortest slubs in samples analyzed, cm.                  | 0.5 | 0.5 | 0.5 | 0.2 | 0.5 | 0.5 | 0.2 | 0.5 |
| Average denier ratio of slub to base yarn                | 3.3 | 3.4 | 4.4 | 3.6 | 2.4 | 1.8 | 2.2 | 3.7 |
| Average interval length between two slubs, cm.           | 208 | 238 | 322 | 370 | 227 | 54  | 104 | 196 |
| Percentage of slub interval having a length greater than |     |     |     |     |     |     |     |     |
| (a) Average interval length                              | 41  | 44  | 48  | 47  | 42  | 46  | 43  | 44  |
| (b) 0.5 × average interval length                        | 69  | 64  | 66  | 61  | 67  | 72  | 76  | 67  |
| (c) 0.2 × average interval length                        | 83  | 87  | 78  | 82  | 85  | 81  | 92  | 79  |
| (d) 1.5 × average interval length                        | 19  | 26  | 27  | 29  | 23  | 18  | 19  | 24  |
| (e) 2.0 × average interval length                        | 12  | 16  | 18  | 21  | 15  | 13  | 11  | 17  |
| <i>d</i> value, mm.                                      | 17  | 13  | 19  | 8   | 3   | 6   | 7   | 4   |

## EXAMPLE 19

The slab yarn obtained by the process of Example 2 was woven into warp of polyethylene oxybenzoate yarn (50 deniers/36 filaments) having no slub, by using an embodiment of the water jet loom as shown in FIG. 13.

Average denier of slubs in the slab yarn was about 510 deniers.

The dimensional value of the water jet loom used and the weaving conditions were as follows:

Inside diameter of the guides: 4 mm.

Inside diameter of water nozzle: 20 mm.

Tension between tenter and a pair of feed rolls: 0.01 g./denier

Rotating speed of the crank shaft of the loom: 350 r.p.m.

Space between nip devices: 20 mm.

Warp density: 120 yarns/inch

Weft density: 70 yarns/inch

The woven fabric had an appearance similar to shantung fabric, on the surface of which there is projected no rough nap. Such effect is desirable for the commercial use and is obtainable from the fact that the water absorbed in the yarn enables the loops to adhere to the yarn when the yarn is picked into shed during the weaving operation and to prevent the nap from projecting on the surface of the resultant fabric. There was hardly experienced any breakage of the slab yarn during the weaving operation by using the yarn as a weft.

We claim:

- 50 3. The process as defined in claim 1 wherein the compressive gas is jetted into the chamber of the hood.
- 4. A process of claim 1 wherein the pressure of the compressive gas is at least 0.5 kg./cm.<sup>2</sup>.
- 55 5. A process for producing a slab yarn which includes the steps of:
  - a. jetting a stream of compressive gas into a hood having a hole at the apex thereof to deflect at the apex and to escape backwardly,
  - b. feeding a multifilament yarn in the deflected stream of gas to fold back the filaments on themselves at the apex of the hood, and
  - c. withdrawing the yarn from the deflected stream of gas through the hole in the hood, at a rate at least 0.5 percent less than the rate of feed, so that the yarn passes through the deflected stream of gas in a countercurrent direction to form slubs composed of filament loops consolidated into the yarn by filament entanglement.
- 60 6. The process as defined in claim 5 wherein the false twisting is performed by passing through a vortex of a compressive gas.
- 65 7. The process as defined in claim 5 wherein the false twisting is performed by passing through a moving friction means in friction contact with the surface of said moving friction means.

UNITED STATES PATENT OFFICE  
CERTIFICATE OF CORRECTION

Patent No. 3,591,955

Dated July 13, 1971

Inventor(s) Shiro Fujita, Jusuke Ushiki, Nagao Nishizawa, Seiji Okawa,  
Kunio Sekiya and Hiroshi Kadowaki

It is certified that error appears in the above-identified patent  
and that said Letters Patent are hereby corrected as shown below:

The name of the assignee is incorrectly stated  
as Nippon Rayon Co.Ltd. whereas the assignment records  
show a merger of Nippon Rayon Co.Ltd. to Unitika Ltd.

Signed and sealed this 21st day of March 1972.

(SEAL)  
Attest:

EDWARD M.FLETCHER,JR.  
Attesting Officer

ROBERT GOTTSCHALK  
Commissioner of Patents